

## UNITED STATES PATENT OFFICE

2,569,122

## LUBRICANT

David E. Adelson, Berkeley, Calif., assignor to  
 Shell Development Company, San Francisco,  
 Calif., a corporation of Delaware

No Drawing. Application December 22, 1947,  
 Serial No. 793,329

12 Claims. (Cl. 252—48.4)

1

This invention relates to novel reaction products having properties of greatly improving and stabilizing lubricants. This invention also pertains to lubricants, such as mineral lubricating oils, synthetic lubricants of hydrocarbon or non-hydrocarbon origin, and the like, containing therein a multi-functional additive having detergent and anti-ringsticking properties, as well as acting as an inhibitor of oxidation and corrosion.

It is well known that various lubricants whether doped or undoped, tend to oxidize and to form corrosive bodies and sludge, when used in modern engines and machines operating under ordinary conditions or at high speeds, elevated temperatures, heavy loads and/or other adverse conditions. Some of the deterioration products of lubricants formed during their use are hard carbonaceous materials which adhere to metal surfaces and cause scratching and scuffing of movable metal parts and the sticking of valves and piston rings in engines. In addition, presently known lubricants are generally incapable of maintaining a continuous lubricating film between movable metal parts, resulting in gradual or rapid wearing away of metal parts. The damage thus caused required replacement of such parts or even the complete overhauling of engines and machines, resulting in expensive loss of production and time.

In the case of the highest quality non-corrosive, stable lubricating oils, which have been highly refined for specific uses, or synthetic lubricants developed for specific or special uses, it has been observed that such oils or lubricants are generally highly susceptible to oxidation and deterioration, becoming progressively more corrosive in engines and machines even under ordinary operating conditions.

To improve the lubricating properties of oils and synthetic lubricants it has become the practice to blend with various lubricants, one and in most cases more than one addition agent, which additives have the effect or property of inhibiting deterioration of lubricants and impart to them certain beneficial properties. Thus, additives have been specifically designed which have the property of inhibiting corrosion of alloyed bearings such as copper-lead, cadmium-silver and the like, developed for automotive, diesel and aircraft engines. Acidic oxidation or decomposition components formed in lubricants during use readily attack these bearings but are inhibited or prevented from doing this by the formation of a corrosion protective film formed on the bearing surface with the aid of the additive. Additives have also been developed which possess the property of modifying the carbonaceous ma-

2

terials formed, by deterioration of lubricants, on piston rods, rings and valves, and other metal parts in internal combustion engines, automotive and truck engines, aviation engines, high speed diesel engines and the like. Such additives serve a very important function because, by modifying this carbonaceous material so that it can be removed easily, the tendency of engine parts to become stuck is inhibited so that ringsticking, piston scuffing, scratching and wearing away of other engine parts and material reduction of engine efficiency, are prevented or materially inhibited.

Other additives have been developed for the purpose of acting as detergents in lubricants in order to assist in the removal of soot or sludge, varnish, lacquer formed from deterioration of the oil when subjected to high operating temperatures. Detergents due to their cleaning action prevent the build up of these deleterious materials and assist in removing those formed. Anti-wear additives have the property of reducing friction of movable metal parts of the same or different metals. Due to the function exerted or property imparted by such additives on lubricants, wear caused by direct frictional contact of metals can be greatly reduced. Also, additives have been developed to withstand extreme pressures, disperse impurities, solubilize certain additives and the like.

The development of numerous additives has been due to the fact that most, if not all additives are capable of functioning in substantially only one specific manner. Very few lubricant additives have the ability of improving a lubricant in more than just one respect. Thus a good antioxidant might not be able to inhibit lacquer and varnish formation on piston rods or act as a detergent or corrosion inhibitor. In many cases it is found that an additive possesses very good properties in one respect, but is the cause of harmful formations and therefore detrimental as an additive in another respect. Therefore, other additives are frequently required to obtain a good stable lubricant. The combination of additives in lubricants wherein each additive exerts its influence without interfering with the function of other additives is a difficult matter to attain. In most cases additives co-react or interfere with each other. To prevent this great care must be taken in selecting the additives, mixing them in specific proportions and continuously watching and replacing additives which have stopped functioning or have deteriorated.

It is an object of this invention to improve the lubricating properties of various lubricating bases by the addition thereto of a minor amount

of a multi-functional material. Another object of this invention is to add to compounded or doped lubricants a multi-functional material whereby a synergistic effect is produced, resulting in a product of accentuated and improved properties. Another object of this invention is to add to oleaginous materials, mineral lubricating oils, synthetic lubricants and the like, a multi-functional material so as to inhibit oxidation and corrosion and prevent the formation of sludge, varnish and lacquer in said lubricants even under adverse operating conditions. Still another object of this invention is to use in lubricating compositions, a multi-functional material which prevents ringsticking as well as the sticking of other engine parts due to deterioration of the lubricant. Also it is an object of this invention to use in oleaginous materials, e. g. in lubricating compositions, a multi-functional material which inhibits wear, scuffing, scratching and other damage to engine parts. Furthermore it is an object of this invention to provide novel multi-functional improving and enhancing additives for lubricating bases. Other objects of this invention will appear as the description proceeds.

To the accomplishment of the foregoing and related ends, this invention consists of features which will be hereinafter fully described, and particularly pointed out in the claims, the following description setting forth in detail certain embodiments of the invention, these being illustrative of but a few variations in which the principle of the invention may be employed.

Broadly stated, this invention is directed to the use, in lubricants of peroxide catalyzed reaction products of organic compounds having an unsaturated linkage or linkages between two or more atoms, with reactive polyhalogenated organic compounds. Another embodiment of this invention is to form a peroxide catalyzed reaction product of organic compounds having an unsaturated linkage or linkages between two or more atoms, with reactive polyhalogenated organic compounds, and thereafter treating said reaction products with hydrogen sulfide in the presence of ammonium hydrosulfide. The above reaction products may be used as such or neutralized with metals or organic bases to form salts thereof and added in minor amounts to a desired lubricant. Among the organic compounds which can be used to form reaction products of this invention are:

I. Unsaturated hydrocarbon compounds:

A. Ethylene, propylene

Butene-1  
Butene-2  
Trimethyl ethylene  
Methylethyl ethylene  
Isobutylene  
Diisobutylene  
Triisobutylene  
The amylenes  
Pentene-2  
Butadiene  
Pentadiene  
3-butadiene  
2-cyano-1,3-butadiene  
2,3-dimethyl-1, hexylene  
Di butylene  
Heptylene  
Isoheptenes  
Isooctenes  
2-ethyl-1-hexene  
1-octene  
2-octene

10  
15  
20  
25  
30  
35  
40  
45  
50

55  
60  
65

70  
75

2-methyl-1-pentene

4-methyl-2-pentene

1-decene

1-dodecene

1-cetene

1-octadecene

Olefinic hydrocarbons, e. g. wax olefins;  
Olefin obtained by decarbonylation of oleyl alcohol or such unsaturated alcohols as are obtained by carboxyl reduction of sperm alcohol;  
Olefins obtained by dehydration of high molecular weight saturated alcohols, etc.

B. Acetylenes—

Butine  
Crotonylene  
Pentine  
Valerylene  
Hexine  
Hexylene  
Heptine  
Phenyl acetylene  
Oenanthyldiene  
Octine  
Caprylidene  
Decine  
Menthene  
Dodecylidene

and their homologues and analogues.

C. Cyclic type hydrocarbons—

Cyclopentane  
Cyclopentadiene  
Cyclohexene  
1-ethylcyclopentene-1  
1,2-dimethylcyclopentene-1  
1-methyl-2-ethylcyclohexene-1  
1,3-dimethylcyclohexadiene-1,3  
1-cyclopentylcyclopentene-1  
Cyclo-octene  
Cyclobutene  
Cyclobutylene  
Cyclohexadiene  
Cyclopropene  
Cycloheptadecene  
Cycloheptatriene  
Cyclo-octadiene, etc.

D. Cyclic terpenes—

|             |                    |
|-------------|--------------------|
| Cymene      | Penchene           |
| Limonene    | Linonene           |
| Pinene      | Sabinene           |
| Bornylene   | Thujene            |
| Methene     | Terpinene          |
| Terpin      | Cadinene           |
| Terpinolene | Clovene            |
| Camphene    | Diterpenes         |
| Carene      | Polyterpenes, etc. |

E. Aromatic type hydrocarbons—

|                        |  |
|------------------------|--|
| Benzene                |  |
| Naphthalene            |  |
| Anthracene             |  |
| Phenanthracene         |  |
| Biphenyl               |  |
| Diphenylalkenes        |  |
| Stibene                |  |
| Diphenylalkanes, e. g. |  |
| Diphenyl methane       |  |
| Alpha-methyl styrene   |  |
| Phenylacetylene        |  |
| Phenyl propyne-1, etc. |  |

70 Compounds under group I, A to E, may contain substituent groups such as alkyl, hydroxy, amine, nitro, nitroso, halogen, carboxyl, mercapto, cyano, etc.

II-A. Polymeric and co-polymeric compounds obtained by polymerizing compounds under group

I-A to E and mixtures thereof. Specific preferred polymeric compounds are:

Ethylene polymers  
Isobutylene polymers  
Butene polymers  
Butadiene polymers  
Polymeric material obtained from cracked gasoline fractions  
Polymeric materials obtained from cracked paraffin waxes  
Polymeric materials obtained from recycle stock from petroleum cracking operation  
Polymers obtained by dehalogenating wax olefines  
Polymers obtained by destructive hydrogenation of rubber olefin polymers obtained from dehalogenating long chain alkyl halides, etc.

B. Polymers obtained from alkene halides, e. g.

Vinyl halides  
2-halo-propylene  
Crotylhalides  
Allylhalides  
2-methyl-3-chloropropene  
Methallyl chloride  
2-ethyl-3-bromopropene  
2-phenyl-3-chloropropene  
2-naphthyl-3-chloropropene  
Vinyl halides  
Crotyl halides  
3-halo-cyclohexene  
2-halo-1,4-diphenyl butene-2  
3-halo-1,4-pentadiene, etc.

C. Copolymers of non-oxygen and of oxygen-containing polymers e. g. polymers of vinyl chloride with either vinyl acetate, furmaric esters, maleic esters, vinylidene chloride; polymers of ethylene with amylene, styrene, stilbene, vinyl acetate, meta acrylic esters, ethyl itaconate, diethyl citraconate, diethylmaleate, diethylfumarate, maleic anhydride, vinylbutyl ether; chloroprene-isobutylene copolymer, butadiene-isobutylene copolymer, reaction product with maleic anhydride, polymethallyl chloride or copolymer thereof with isobutylene, etc.

III. Saturated alkyl mono-carboxylic acids (the required unsaturation linkage being the carboxyl group



A.

|           |                    |
|-----------|--------------------|
| Capric    | Lignoceric         |
| Undecylic | Cerolic            |
| Lauric    | Monotanic          |
| Myristic  | Melisic            |
| Palmitic  | Ethyl butyric      |
| Stearic   | Ethyl hexoic, etc. |
| Arachidic |                    |

B. Unsaturated alkyl monocarboxylic acids—

|                   |                             |
|-------------------|-----------------------------|
| Acrylic           | Clupanodonic acid           |
| Butenic           | Linolenic                   |
| Crotonic          | Brassidic                   |
| Pentenic          | Elaidic                     |
| Tiglic            | Corn oil acid               |
| Hexenic           | Lard oil acids              |
| Teracrylic        | Soy oil acids               |
| Hypogallic        | Tung oil acids              |
| Oleic             | Elacostearic                |
| Linoleic          | Stearoleic                  |
| Erucic            | Cocoanut fatty acids        |
| Hexylacrylic acid | Co. tonseed oil acids, etc. |
| Hexadecene acid   |                             |

C. Hydroxy alkyl carboxylic acids (required unsaturated linkage being the



group or  $\text{C}=\text{C}$ )—  
Dimethyl hydroxy caprylic  
Dimethyl hydroxy capric  
Hydroxy phytoleic  
Ricinoleic  
Ricinelaic  
12-hydroxy stearic  
9,10-dihydroxy stearic  
4-hydroxy palmitic  
Linusic  
Sativic  
Lanoceric  
Dihydroxy gadoleic  
Dihydroxy behenic  
Quince oil acids, etc.

D. Keto acids (required unsaturated linkage being the  $\text{C}=\text{O}$  group)—

|                 |                            |
|-----------------|----------------------------|
| Pyronacenic     | Licanic                    |
| Propanyl formic | 12 keto stearic            |
| Butyryl formic  | 13 keto behenic acids, etc |
| Aceto butyric   |                            |

E. Aldehyde alkyl carboxylic acids (required unsaturated linkage being the  $\text{C}=\text{O}$  group or the  $\text{C}=\text{C}$ )—

|                        |  |
|------------------------|--|
| Aldovaleric            |  |
| Formylacrylic          |  |
| Mucolronic acids, etc. |  |

F. Polycarboxylic alkyl acids (required unsaturated linkage being the  $\text{C}=\text{O}$  group or the  $\text{C}=\text{C}$ )—

|                                             |  |
|---------------------------------------------|--|
| Cycloalkylene, alkylene, arylalkyl malonic  |  |
| Cycloalkylene, alkylene, arylalkyl succinic |  |
| Cycloalkylene, alkylene, arylalkyl glutaric |  |
| Cycloalkylene, alkylene, arylalkyl adipic   |  |
| Pimelic                                     |  |
| Azelic                                      |  |
| Brassylic                                   |  |
| Alkylene maleic                             |  |
| Furmaric                                    |  |
| Itaconic                                    |  |
| Citraconic                                  |  |
| Mesaconic                                   |  |
| Glutaconic                                  |  |
| Tartaric                                    |  |
| Malic                                       |  |
| Aspartic                                    |  |
| Mesoxalic                                   |  |

Tricarballytic acids and homologs, e. g.

55      Aconitic  
Tartaric  
Citric acids, etc.  
The alkyl group of the acid preferably should contain at least 6 carbon atoms.

60      G. Miscellaneous alkyl acids—

Acidic products produced by oxidation of hydrocarbons, e. g.

|                                                                      |  |
|----------------------------------------------------------------------|--|
| Olefinic paraffin wax, etc;                                          |  |
| Mercapto oleic                                                       |  |
| Mercapto stearic                                                     |  |
| Thio stearic                                                         |  |
| Cetyl alpha amino succinic                                           |  |
| Amino caprylic                                                       |  |
| Mercapto succinic                                                    |  |
| Cetyl amino succinic                                                 |  |
| Phosphonato fatty acids e. g., phosphonato butyric to stearic acids; |  |
| Cyano fatty acids, e. g., cyano butyric to stearic acids             |  |

These phosphonato and cyano acids may also include the polycarboxylic acids e. g. phosphonato alkyl succinic acid, etc.

Either or both of the oxygen atoms in the carboxylic acid radical of A to G may be replaced by sulfur, selenium, and/or tellurium atoms resulting in the following acid radicals: CXOH, COXH, CXXH, wherein X is sulfur, selenium or tellurium. Also these acids may contain substituent groups attached in appropriate position of the acid molecule so as to aid in solubilizing and enhancing their lubricating properties.

IV. Aromatic acids, represented by the general formula



wherein Ar is an aromatic nucleus; X' and X may be non-polar or polar radicals attached to the aryl nucleus; Z is a carboxylic acid group such as CYYH wherein either or both Y's may be oxygen, sulfur, selenium or tellurium, said acid being attached directly to the aryl nucleus or linked to it through X; m may be zero or an integer of from 1 to 3; n may be zero or one and y may be an integer of 1 or 2. Representative acids are:

Benzoic

Phthalic

Toluic

Xylic

Phenyl fatty acids, e. g.

Phenyl acetic to phenyl stearic acids

Benzyl acetic to benzyl stearic acid

Cinnamic acid

Salicylic acid

Mendelic acid

Phenyl glyoxylic

Benzoyl propionic acid

Phenyl laevulunic acid

Phenyl alkyl succinic acid

Benzyl alkyl succinic acid

Phenyl alkyl glutaric acid

o-Vinyl benzoic acid

Phenyl angelic acid

Naphthoic acid

Naphthyl stearic acid

Anthranilic acid

Phenyl cinnamic acid

Methyl cinnamic acid

Methoxy cinnamic acid

Atropic acid

Phenyl crotonic acid

Phenyl amino crotonic acid

Phenyl acrylic acid

Phenyl ricinoleic acid

Benzal lactic acid

Benzal malonic acid

Benzal propionic acid

Mercapto (phenyl, tolyl, xylyl, xenyl, naphthyl anthracyl) fatty acids e. g.—

Phenyl mercapto acetic to phenyl mercapto stearic acid

Ethyl mercapto phenyl acetic acid

Aryl mercapto benzene-4-carboxylic

#### V. Cyclic acids:

Naphthenic acids derived from petroleum hydrocarbons—

Cyclohexane carboxylic acid

Hexahydrobenzoic acid

Tetra hydrotoluic acid

Alkyleno cyclohexadiene carboxylic acid

Abietic acid

- Alkyl hexahydrophthalic acid  
Camphane-3-carboxylic acid  
Camphoric acid and derivatives  
Cholic acid and derivatives  
Cholic acid  
Laurolenic acid  
Chaulmoogric acid  
Tetrahydrobenzoic acid  
Tetrahydrophthalic acid  
Dihydrophthalic acid  
Tetrahydroxylic acid  
Fural acrylic acid  
Linseed oil fatty acid  
Oiticica acid  
Cyclohexylacetic acid  
Cyclohexylbutyric acid  
Cyclohexylcaproic acid  
Cyclohexyl propionic acid  
Cyclohexyl valeric acid  
Fencholic acid, etc.

#### VI. Heterocyclic acids represented by the general formula



wherein Q is a five or six-membered heterocyclic ring; R' and R may be alkyl, aryl alkaryl, aryl-alkyl alkoxy; aryloxy radicals; Z is a carboxyl radical, m may be zero or an integer of 1 and 2 and n may be zero or 1 and y may be an integer of 1, 2 or 3. Specific heterocyclic acids may include:

- Picolinic acid  
35 Nicotinic acid  
Isonicotinic acid  
Quinolinic acid  
Cinchomeronic acid  
Lutidinic acid  
40 Berberonic acid  
Alpha- and beta-carbo cinchomeronic acid  
Quinic acid  
Cynchomeronic acid;  
Pyrole carboxylic acids;  
45 Quinoline carboxylic acids;  
Thiazole carboxylic acids;  
Thiophene carboxylic acids; etc.

#### VII. I-G miscellaneous acids such as:

##### 50 Xanthtic acids



##### 55 Thio xanthtic acids



##### Carbamic acids



##### 60 Thiocarbonic acids



##### 65 Thio carbamic acids



##### 70 Thio carbamic acids



## Dithio carbamic acids



wherein R is represented by alkyl, aryl, arylalkyl, alkylaryl cyclo radicals and the like. Some specific compounds may be:

Butyl mono and dithio carbamic acid  
 Diethyl mono and dithio carbamic acid  
 Dimethyl mono and dithio carbamic acid  
 Diethyl mono and dithio carbamic acid  
 Dioctyl mono and dithio carbamic acid  
 Dipropyl mono and dithio carbamic acid  
 N-ethyl-N-phenyl mono and dithio carbamic acid  
 Octyl-butyl mono and dithio carbamic acid  
 Dicyclohexyl mono and dithio carbamic acid  
 Methyl-octyl mono and dithio carbamic acid  
 Dibenzyl amyl dithiocarbamic acid, etc.

Included under miscellaneous acids of group VII may be the acid anhydrides and acid halides such as:

## Acid anhydrides—

Acrylic  
 Butenic  
 Crotonic  
 Pentenic  
 Tiglic  
 Hexenic  
 Teracrylic  
 Hypogallic  
 Oleic  
 Linoleic  
 Erucic  
 Hexylacrylic acid  
 Acid anhydride e. g. acrylic acid anhydride  
 Linolenic  
 Brassidic  
 Elaidic  
 Corn oil acid  
 Lard oil acids  
 Soy oil acids  
 Tung oil acids  
 Elacostearic  
 Stearoleic  
 Cocoanut fatty acids  
 Cottonseed oil acids, etc.

## Acid halides—

Acrylic  
 Butenic  
 Crotonic  
 Pentenic  
 Tiglic  
 Hexenic  
 Teracrylic  
 Hypogallic  
 Oleic  
 Linoleic  
 Erucic  
 Hexylacrylic acid  
 Acid halide, e. g. acrylic acid halide  
 Linolenic  
 Brassidic  
 Elaidic  
 Corn oil acid  
 Lard oil acids  
 Soy oil acids  
 Tung oil acids  
 Elacostearic

## Stearoleic

Cocoanut fatty acids  
 Cottonseed oil acids, etc.

## 5 VIII. Organic compounds containing an inorganic acid:

- A. Sulfonic acids—  
 Benzene sulfonic acid  
 Toluene sulfonic acid  
 10 Tri isopropyl naphthalene sulfonic acid  
 Diphenyl sulfonic acid  
 Polyalkyl aromatic sulfonic acid, e. g. poly amyl naphthalene sulfonic acid  
 Diwax benzene sulfonic acid  
 15 Xylene sulfonic acid  
 Benzene disulfonic acid  
 Alkane sulfonic acids, e. g. amyl, octyl, nonyl, lauryl, dodecyl sulfonic acids  
 20 Petroleum sulfonic acids derived from various petroleum fractions such as—  
 Gas oil  
 Kerosene  
 Light oil  
 25 Turbine oil  
 Mineral lubrication oil  
 Heavy oil  
 Petroleum waxes, e. g.  
 Petrolatum  
 30 Paraffin wax and mixtures of various hydro-carbon fractions  
 Wax sulfo salicylic acid  
 Diwax naphthalene sulfonic acids, etc.

## 35 IX. Phosphorus-containing acids:

- Substituted phosphorus acids containing an organic substituent: the aliphatic, cyclo aliphatic and aromatic acid esters of phosphoric acid, thio phosphoric acids, phosphorus acids and thio phosphorus acids. These are obtained by reacting  $\text{POCl}_3$ ,  $\text{P}_2\text{O}_5$ ,  $\text{PCl}_3$ ,  $\text{P}_2\text{S}_3$ ,  $\text{P}_2\text{S}_5$ ,  $\text{P}_4\text{S}_7$ ,  $\text{Br}$  with any of the acids of groups I, A-E, II, A-C, III, A-G, IV, V, VI, and VII. These inorganic phosphorus compounds may also be reacted with any of the materials listed under groups X, XI, XII, 45 and XIII, as well as esters which may be formed by reacting the alcohols of groups X and/or XI with the acids of groups III, IV, V, VI and VII.

X. Alcohols and thio alcohols such as  $\text{RXH}$  where  $\text{X}$  is O, Se, Te and S and R represents 50 alkylene, cyclo-alkylene, aralkyl radical or derivatives thereof.

## A. Aliphatic—

- |                  |                   |
|------------------|-------------------|
| Vinyl alcohol    | 2-propyn-1-ol     |
| 55 Alkyl alcohol | Oleyl alcohol     |
| Geraniol         | Wood fat alcohol  |
| Citronellol      | Olefinic wax      |
| Linalool         | Alcohol           |
| Farnesol         | Methallyl alcohol |
| 60 Phytol        | Allyl alcohol     |

## B. Cyclic alcohols—

- |                           |  |
|---------------------------|--|
| Cyclohexanol              |  |
| Alkyl cyclohexanol, e. g. |  |
| 65 Methyl cyclohexenol    |  |
| Amyl cyclohexenol         |  |
| Cyclobutanol              |  |
| Naphthenic alcohol, etc.  |  |

## 70 C. Aromatic alcohol—

- |                                    |  |
|------------------------------------|--|
| Benzyl                             |  |
| Phenyl ethyl                       |  |
| Dibenzyl                           |  |
| Toly                               |  |
| Phenyl octyl                       |  |
| 75 Octadecyl benzyl alcohols, etc. |  |

## D. Natural occurring alcohols and synthetic alcohols—

Alcohols as found in wool fat, sperm oil  
Alcohols produced by oxidation of hydrocarbons, e. g.

Paraffin wax  
Sweat wax  
Petrolatum  
and the like

## XI. Phenolic compounds—

(R—Ar—X—H)

wherein Ar is an aryl nucleus, X is O, S, Se, Te and R is a substituent non-polar and/or polar group and/or groups.

Phenol

Alkylene phenol

Dibutyl phenol and its thio phenols

Amyl phenol and its thio phenols

Tertiary butyl

p-Tertiary amyl

Octylene

p-Iso-octylene

Isobutylene

Nonylene

Cetyl phenols and thio phenols

Alkylamino phenol

Alkyl amino naphthol

Catechol

Resorcinol

Pyrogallol

All of these compounds may contain substituent groups as listed in column 14 and the like. Substituted products are: hydroquinone, quinone, orcinol, phloro-glucinol, cresols, thymol, saligenin, cinnamyl alcohol, methyl phenyl carbinol, eugenol, cardanols, etc. Also the thio phenolic derivatives of these phenolic compounds may be used as well as various reaction products thereof such as obtained by reacting phenolic compounds with:  $\text{SCl}_2$ ,  $\text{S}_2\text{Cl}_2$ , S,  $\text{SO}_2$  and the like to form sulfide derivatives which may be represented broadly by the formula:



wherein Ar is an aryl nucleus, R is an alkyl, aralkyl radical and the like, X is S which in turn can be replaced by O, Se or Te in whole or in part, and u is an integer of from 1 to 4, and Y may be a polar radical such as listed under VII B either or both m and n may be zero or an integer of 1 or 2.

Phenolic condensation products may also be formed by reacting products under group IX with aldehydes of the aliphatic, aromatic or cyclic type, specifically represented by formaldehyde, acetaldehyde, crotonaldehyde, butyraldehyde, benzaldehyde; furaldehyde and the like. The condensation reaction is carried out at rather an elevated temperature using an acid or basic catalyst. Typical condensation reaction products may be formed between:

Octyl phenol-formaldehyde  
Octyl phenol-acetaldehyde  
Iso octyl phenol-acetaldehyde  
Iso octyl phenol-crotonaldehyde  
Octyl phenol-benzaldehyde  
Octyl phenol-furaldehyde  
Octyl thio phenol-furaldehyde  
Octyl thio phenol-formaldehyde  
Amyl phenol-formaldehyde  
Amyl phenol-furaldehyde

## XII. Aldehydes:

## A. Aliphatic (saturated and unsaturated)—

Acetaldehyde  
Propionaldehyde  
5 Butyraldehyde  
Caproaldehyde  
and the like;  
Acrolein

## 10 B. Aromatic—

Benzaldehyde  
Cinnamaldehyde  
Salicylaldehyde

## 15 XIII. Ketones:

## A. Aliphatic (saturated and unsaturated)—

20 Acetone  
Butanone  
Hexanone  
Oleone  
Palmitone  
Methyl ethyl ketone  
Methyl propyl ketone  
25 Butyrone  
Butenone  
Vinylethyl ketone  
Pantanone

## 30 B. Aromatic—

Acetophenone  
Propiophenone  
Dibenzyl ketone

## C. Cyclic ketones:

Cyclobuteneone  
Cyclopentenone  
Quinones  
Cycloheptenone

40 Pure isophorone  
and isophorone bottoms the manufacture of  
which is fully described hereinbelow

Cyclohexenone

Carvomenthone

Menthone

Pulegone

Carvone

Muscone

Isophorone bottoms are primarily high molecular weight unsaturated ketones having at least 12 and preferably more than 18 carbon atoms in the molecule. These products may be obtained by condensation of acetone in a caustic solution under elevated temperature and pressure. Specifically the product is obtainable by condensing acetone in a 30% to 60% caustic solution at a temperature ranging between about 130° C. and about 170° C., and under a pressure of from about 300 to about 500 pounds per square inch.

The resultant product is subjected to distillation to remove distillable ketones and other constituents and impurities. The product remaining in the still is preferably purified by filtration, solvent treatment, and comprises crude unsaturated cyclic ketones of high molecular weight, preferably referred to as "crude isophorone bottoms." The term "isophorone bottoms" as referred herein is usually a complex mixture of high molecular weight unsaturated

70 cyclic ketones containing at least 12 and preferably more than 18 carbon atoms in the molecule. The product thus formed is not to be confused with straight isophorone which is specifically 3,5,5 - trimethyl cyclohexene - 2 - one - 1, 75 which is an unsaturated cyclic ketone contain-

ing only nine carbon atoms in the molecule. Isophorone bottoms produced by condensation of acetone under conditions referred to above includes within its scope any and all unsaturated cyclic ketones containing at least 12 and preferably more than 18 carbon atoms and having generally the chemical structural configuration of isophorone as well as the chemical structural configuration resulting from its further condensation.

Crude isophorone bottoms can be fractionated and/or chemically treated and each fraction therefrom can in turn be treated with a peroxide catalized polyhalo organic compound and thereafter treated with  $H_2S-NH_4HS$  if desired to produce one of the additives of this invention. Among the various fractions which can be obtained from crude isophorone bottoms are topped, crude isophorone bottoms which contain at least 18 carbon atoms in the molecule and are obtained after removal of distillate from crude isophorone bottoms to a still head temperature of  $140^\circ C.$  at 10 mm. mercury pressure. Another fraction of crude isophorone bottoms can be subjected to hydrolysis with dilute sodium hydroxide and the acetone and isophorone formed removed by distillation. The bottoms can then be filtered and purified and comprise essentially unsaturated cyclic ketones containing at least 12 or more carbon atoms in the molecule and are referred to as crude, hydrolyzed isophorone bottoms. This material can be subjected to distillation to split it into two fractions. The distilled hydrolyzed isophorone fraction has a boiling point of about  $140^\circ C.$  at 10 mm. mercury pressure and consists of a mixture of unsaturated cyclic ketones containing between 15 to 18 carbon atoms in the molecule. The residue is referred to as topped, crude hydrolyzed isophorone bottoms and is similar to topped crude isophorone bottoms. This residue comprises essentially unsaturated cyclic ketones of at least 15 carbon atoms and higher in the molecule. Crude isophorone bottoms can be also subjected to condensation over solid sodium hydroxide to yield two types of resinous materials. The first resinous fraction or soft resin has a viscosity at  $210^\circ F.$  of about 25-26 centistokes and an average molecular weight of from 320 to 250. The heavier fraction or medium resin has a viscosity at  $210^\circ F.$  of about 25-26 centistokes and an average molecular weight of from 320 to 350. The heavier fraction or medium resin has a viscosity at  $210^\circ F.$  of about 80 to 120 centistokes and an average molecular weight of from 370 to 390. The unsaturated cyclic ketones can be hydrogenated to produce saturated cyclic ketones. All of the various saturated and unsaturated cyclic ketone fractions obtained in the manner described above can be used.

XIV. Natural fats, oils and waxes and their derivatives and miscellaneous compounds:

A. Vegetable and animal oils, fats, and waxes such as—

Castor oil  
Cocoanut oil  
Corn oil  
Cottonseed oil  
Horse fat  
Lard oil  
Mutton tallow  
Beef tallow  
Neat's-foot oil

Palm oil  
Peanut oil  
Rapeseed oil  
Soya bean oil  
5 Sperm oil  
Whale oil  
Wool fat  
Japan wax  
Olefin waxes  
10 Paraffin waxes  
Wax tailings  
Petrolatum  
Vegetable and animal phosphatidic materials  
Montan wax  
15 Carnauba wax  
Beeswax  
Spermaceti  
Castor oil distillate  
Ozokerite  
Tall oil  
and the like and fractions and derivatives thereof

XV. Esters:

Esters contemplated for use in this invention may be obtained by reacting any of the compounds listed under groups III, A-6, IV, V, VI, and VII, with compounds of groups X and XI. Specific esters are:

|                      |                                       |
|----------------------|---------------------------------------|
| 30 Allyl acetate     | Methyl acrylate                       |
| Allyl propionate     | Allyl allyloxyacetic acid             |
| Allyl laurate        | Methyl allyl methallyl oxyacetic acid |
| Allyl capronate      | Allyl metallyloxyacetate              |
| 35 Allyl isovalerate | Glyceryl monoricinoleate              |
| Allyl stearate       | Glyceryl monooleate                   |
| Lanyl acrylate       | Allyl succinate                       |
| Methyl crotonate     |                                       |

XVI. Ethers:

The ethers contemplated for use in this invention may be symmetrical, unsymmetrical, or mixed ethers of dialkyl ethers, alkyl-aryl ethers, aryl ethers and the like. Specifically it is desirable to use:

|                                              |                                       |
|----------------------------------------------|---------------------------------------|
| 40 A. Aliphatic (saturated and unsaturated)— |                                       |
| Ethyl vinyl ether                            | Ethyl propargyl, etc.                 |
| Ethyl propenyl ether                         | Divinyl ether                         |
| Methyl isopropenyl ether                     | Diallyl ether                         |
| 50 Ethyl isopropenyl                         | Dicrotyl ether                        |
| Methallyl ether                              | Dimethylallyl ether                   |
| Ethyl allyl ether                            | Diisopropenyl ether                   |
| n-Propyl allyl ether                         | Dihexenyl ether                       |
| 55 Isopropyl allyl ether                     | Allyl (2-methyl-4-pentene-2-yl) ether |
| 4-ethoxy-1-butene                            |                                       |
| 6-ethoxy-1-hexene                            | Allyl linallyl ether                  |

B. Cyclic and poly ethers—

|                 |                      |
|-----------------|----------------------|
| Ethylene oxide  | Acetal               |
| Propylene oxide | Dioxan, and the like |

C. Aromatic ethers—

|                      |                                |
|----------------------|--------------------------------|
| Allyloxyphenyl ether | Benzyl ether                   |
| Anisole              | Cardanoxyethanol               |
| Phenetole            | Allyl-alpha-phenyl vinyl ether |
| 65 Diphenyl          | Dixenyl                        |
| Dixenyl              | Allyl phenyl ether             |
| Dinaphthyl ethers    | and the like.                  |
| Benzyl phenyl ether  |                                |

D. Substituted ethers—

Alkoxy ethers of polyhydroxy aromatics such as:

Resorcinol  
Pyrogallol  
and the like.

**15**  
**REAGENT**

Any of the above compounds and mixtures thereof may be reacted with a polyhalogenated organic compound in the presence of a peroxide catalyst. The polyhalogenated organic compounds may include: carbon tetrachloride, chloroform, methylene chloride, carbon tetrabromide, bromoform, methylene bromide, iodoform, methylene chloroiodide, hexachloroethane, di- and tri-chloroethane polyhalogenated fatty acids in which the halo radicals are preferably attached in the alpha or beta position to the carboxyl radical. Specific compounds are: dichloroacetic acid, trichloroacetic acid, alpha, alpha-dichloropropionic acid, alpha, alpha, beta, beta-tetrachloropropionic acid, alpha, beta-dichloropropionic acid, alpha, alpha-dichlorobutyric acid, alpha, beta-dichlorobutyric acid, alpha, alpha, beta-trichlorobutyric acid, alpha, beta-dichloroisobutyric acid, phenyldichloro acetic acid, dibromo acetic acid, tribromo acetic acid, alpha, alpha-dichloropentanoic acid, alpha, alpha-dibromopentanoic acid, diiodo acetic acid, triiodo acetic acid, beta, beta-dibromopropionic acid, alpha, alpha-dichlorocaprylic acid, etc.

**CATALYSTS**

The peroxide catalysts which can be used to carry out the halogenation reaction may include:

Hydrogen peroxide  
Benzoyl peroxide  
Lauroyl peroxide  
Tetralin peroxide  
Urea peroxide  
Butyrl peroxide  
Diethyl peroxide  
Di-tert-butyl peroxide  
Diacetyl peroxide  
Acetyl benzoyl peroxide  
Propionyl peroxide  
Cyclohexanone peroxide  
Ascaridole  
Alkali and alkaline earth metal peroxides or mixtures thereof can be used

The reaction product of this invention, namely, a peroxide catalyzed reaction product between an organic compound having an unsaturated linkage or linkages and a polyhalogenated organic compound can be carried under reflux conditions for a period of time sufficient for the reaction to go to completion. This is evidenced when hydrogen chloride seems to evolve and may require from a few hours to over 72 hours depending upon the reactants taking part in the reaction, the temperature and the like.

The reaction product of this invention namely a peroxide catalyzed polyhalogenated organic compound can be treated with hydrogen sulfide in the presence of ammonium hydrosulfide to obtain an additive suitable for use as additives in lubricants operating under the most adverse conditions. This reaction can be formed at room or elevated temperatures, preferably in closed vessels. The use of elevated temperatures apparently only speeds up the reaction. However, the cost of fuel and special equipment outweighs this feature, and it has been ordinarily found more advantageous to simply allow the ammonium hydrosulfide-hydrogen sulfide reactions to take place at room temperature in closed vessels for the necessary period of time, e. g. from one week to one month or more, depending upon the organic material being treated. If desired

**16**

this reaction product may be formed in the presence of a suitable inert solvent.

To more clearly illustrate the present invention, the following examples are presented. It is to be understood, however, that various modifications can be resorted to without departing from the spirit of the invention.

**GROUP I**

*Example I*

*Reaction product of peroxide catalyzed, topped, crude isophorone bottoms with carbon tetrachloride.*—Approximately 1 mole of topped, crude isophorone bottoms; 4 moles of carbon tetrachloride and 0.04 mole of benzoyl peroxide were reacted under reflux conditions until the reaction was completed. The excess carbon tetrachloride was removed by distillation. The residue was a dark, viscous material containing 13.5 to 15.4 per cent chlorine.

*Example II*

*Reaction product of peroxide catalyzed cracked wax olefins with carbon tetrachloride.*—Approximately 1 mole of cracked wax olefins having a molecular weight of about 218, a boiling point range of 220-300° C. and the double bond being present in the terminal position were reacted with carbon tetrachloride in the presence of benzoyl peroxide under conditions as described in Example I. Hydrogen chloride was evolved during the reaction period. The reaction product formed was a dark red oil which contained approximately 8.7% chlorine and possessed excellent extreme pressure properties.

*Example III*

*Reaction product of a peroxide catalyzed hexadecene-1 with dichloroacetic acid.*—A solution of approximately 0.5 mole of hexadecene-1, and 0.02 mole di-tertiary butyl peroxide in about 2 moles of dichloroacetic acid were stirred and heated on a steam bath for over 24 hours. The reaction mixture was then dissolved in a non-aromatic hydrocarbon solvent having a boiling range of between about 164° F. and 233° F. and washed with water in order to remove excess dichloroacetic acid. The solvent is removed leaving behind a dark, viscous liquid containing about 14.0% chlorine which possesses excellent extreme pressure properties.

*Example IV*

*Reaction product of peroxide catalyzed topped, crude isophorone bottoms with chloroform.*—Approximately one mole of topped, crude isophorone bottoms and chloroform were reacted in the presence of benzoyl peroxide.

This reaction product in the same manner as described in Example II, except that chloroform was used as the chlorinating agent. The final product was a dark red oil containing about 1.2 to 2.4% chlorine.

*Example V*

*Reaction product of peroxide catalyzed cracked wax olefins with trichloroacetic acid.*—Approximately 0.5 mol of cracked wax olefins, about 2 moles of trichloroacetic acid and 0.02 mols of di-tertiary butyl peroxide was stirred and heated on a steam bath for 24 hours. At the end of the reaction period considerable evolution of hydrogen chloride was noted. The product was dissolved in a non-aromatic solvent as referred to in Example III and excess trichloroacetic acid

washed out by means of water. The solvent was evaporated leaving behind a dark brown liquid having a chlorine content of approximately 20.8 per cent.

*Example VI*

*Reaction product of peroxide catalyzed C<sub>8</sub>-C<sub>18</sub> olefin having non-terminal double bonds with trichloroacetic acid.*—This reaction product was formed in the manner described in Example V except that an olefin of C<sub>8</sub>-C<sub>18</sub> having non-terminal double bonds and a molecular weight above 185 was utilized. The chlorine content of the final product was approximately 25.8%.

Other peroxide catalyzed polyhalogenated organic compounds of this invention are:

1. Reaction product of peroxide catalyzed spray oil and carbon tetrachloride.
2. Reaction product of peroxide catalyzed spray oil and chloroform.
3. Reaction product of peroxide catalyzed hydrogen pressure distillate bottoms and carbon tetrachloride.
4. Reaction product of peroxide catalyzed hydrogen pressure distillate bottoms and chloroform.
5. Reaction product of peroxide catalyzed cracked wax olefins and carbon tetrachloride.
6. Reaction product of peroxide catalyzed cracked wax olefins and chloroform.
7. Reaction product of peroxide catalyzed cracked wax olefins and dichloroacetic acid.
8. Reaction product of peroxide catalyzed isophorone with carbon tetrachloride.
9. Reaction product of peroxide catalyzed isophorone with chloroform.
10. Reaction product of peroxide catalyzed C<sub>8</sub>-C<sub>18</sub> olefin and chloroform.
11. Reaction product of peroxide catalyzed C<sub>8</sub>-C<sub>18</sub> olefin and carbon tetrachloride.
12. Reaction product of peroxide catalyzed oleic acid and carbon tetrachloride.
13. Reaction product of peroxide catalyzed polymeric ethylene and dichloroacetic acid.
14. Reaction product of peroxide catalyzed allyl alcohol and dichloroacetic acid.
15. Reaction product of peroxide catalyzed cyclohexenone and chloroform.
16. Reaction product of peroxide catalyzed castor oil and chloroform.
17. Reaction product of peroxide catalyzed cinnamyl alcohol and carbon tetrachloride.
18. Reaction product of peroxide catalyzed cinnamic acid and carbon tetrachloride.
19. Reaction product of peroxide catalyzed copolymer of butadiene-isobutylene and dichloroacetic acid.
20. Reaction product of peroxide catalyzed copolymer of ethylene-vinyl butyl ether and carbon tetrachloride.
21. Reaction product of a peroxide catalyzed isophorone and trichloroacetic acid.
22. Reaction product of a peroxide catalyzed cracked wax olefin and trichloroacetic acid.

**GROUP II**

*Example VII*

*A. Initial reaction product of peroxide catalyzed, topped, crude isophorone bottoms with carbon tetrachloride.*—Approximately 1 mole of topped, crude, isophorone bottoms; 4 moles of carbon tetrachloride and 0.04 mole of benzoyl peroxide were reacted under reflux conditions until the reaction was completed with required between 24 to 72 hours. The excess carbon tetra-

chloride was removed by distillation. The poly-chlorinated reaction product was a dark viscous material containing approximately 13.5% to 15.4% chlorine.

5. *B. Final reaction product obtained by treating VII-A with H<sub>2</sub>S in the presence of ammonium hydrosulfide.*—Approximately 155 grams of the above reaction product was dissolved in 300 cc. of isopropyl alcohol and admixed with 500 cc. of isopropyl alcohol which had been saturated with ammonium hydrosulfide and hydrogen sulfide. Hydrogen sulfide was passed through the resulting mixture until saturated. The reaction vessel was closed and allowed to stand for one week.
10. The reactor was then opened and the isopropyl alcohol solution was filtered and the solvent removed by evaporation. The residue was dissolved in a non-aromatic hydrocarbon having a boiling range of between about 164° F. and 233° F. and
15. washed with water. The solvent and water are removed by suitable means and the resultant product which was a dark brown viscous material contained 2.2% sulfur and 10.4% chlorine. The product was soluble in mineral oil and had excellent extreme pressure properties.
- 20.
- 25.

*Example VIII*

- A. Initial reaction product of peroxide catalyzed cetene with dichloroacetic acid.*—Approximately 0.5 mole of cetene, 2 moles of dichloroacetic acid and 0.02 mole of di-tert-butyl peroxide were admixed and heated on a steam bath for 24 hours. The reaction mixture was then dissolved in a non-aromatic hydrocarbon having a boiling range of between 164° F. and 233° F. and washed with water to remove excess dichloroacetic acid. After removal of the solvent in vacuo, the product remaining was a dark, viscous liquid containing 14.0% chlorine.
- 30.
- 35.
40. *B. Final reaction product obtained by treating II-A with H<sub>2</sub>S presence of ammonium hydrosulfide.*—The reaction product of II-A was dissolved in isopropyl alcohol and admixed with an approximately equal amount of isopropyl alcohol
45. which has been saturated with ammonium hydrosulfide. Hydrogen sulfide was passed through the resulting mixture until saturated. The reaction vessel was opened, the solvent removed and the residue dissolved in a non-aromatic hydrocarbon and water washed. The solvent and water were removed and the residue contained both sulfur and chlorine and exhibited excellent extreme pressure properties when admixed with lubricants.
- 50.
55. Other peroxide catalyzed polyhalogenated organic compounds or these which have been further treated with ammonium hydrosulfide-hydrogen sulfide to produce reaction products of this invention are:
60. 1. Reaction product of peroxide catalyzed spray oil and carbon tetrachloride treated with hydrogen sulfide-ammonium hydrosulfide.
2. Reaction product of peroxide catalyzed spray oil and chloroform treated with hydrogen sulfide-ammonium hydrosulfide.
65. 3. Reaction product of peroxide catalyzed hydrocarbon pressure distillate bottoms and carbon tetrachloride treated with hydrogen sulfide-ammonium hydrosulfide.
4. Reaction product of peroxide catalyzed hydrocarbon pressure distillate bottoms and chloroform treated with hydrogen sulfide-ammonium hydrosulfide.
70. 5. Reaction product of peroxide catalyzed cracked wax olefins and carbon tetrachloride
- 75.

treated with hydrogen sulfide-ammonium hydro-sulfide.

6. Reaction product of peroxide catalyzed cracked wax olefins and chloroform treated with hydrogen sulfide-ammonium hydrosulfide.

7. Reaction product of peroxide catalyzed cracked wax olefins and dichloroacetic acid treated with hydrogen sulfide-ammonium hydro-sulfide.

8. Reaction product of peroxide catalyzed isophorone with carbon tetrachloride treated with hydrogen sulfide-ammonium hydrosulfide.

9. Reaction product of peroxide catalyzed isophorone with chloroform treated with hydrogen sulfide-ammonium hydrosulfide.

10. Reaction product of peroxide catalyzed wax olefin and chloroform treated with hydrogen sulfide-ammonium hydrosulfide.

11. Reaction product of peroxide catalyzed wax olefin and carbon tetrachloride treated with hydrogen sulfide-ammonium hydrosulfide.

12. Reaction product of peroxide catalyzed oleic acid and carbon tetrachloride treated with hydrogen sulfide-ammonium hydrosulfide.

13. Reaction product of peroxide catalyzed polymer ethylene and dichloroacetic acid treated with hydrogen sulfide-ammonium hydrosulfide.

14. Reaction product of peroxide catalyzed allyl alcohol and dichloroacetic acid treated with hydrogen sulfide-ammonium hydrosulfide.

15. Reaction product of peroxide catalyzed cyclohexenone and chloroform treated with hydrogen sulfide-ammonium hydrosulfide.

16. Reaction product of peroxide catalyzed castor oil and chloroform treated with hydrogen sulfide-ammonium hydrosulfide.

17. Reaction product of peroxide catalyzed cinnamyl alcohol and chloroform treated with hydrogen sulfide-ammonium hydrosulfide.

18. Reaction product of peroxide catalyzed cinnamyl acid and chloroform treated with hydrogen sulfide-ammonium hydrosulfide.

19. Reaction product of peroxide catalyzed co-polymer of butadiene-isobutylene and dichloroacetic acid treated with hydrogen sulfide-ammonium hydrosulfide.

20. Reaction product of peroxide catalyzed co-polymers of ethylene vinyl butyl ether and carbon tetrachloride treated with hydrogen sulfide-ammonium hydrosulfide.

Reaction product of this invention may be neutralized with a suitable metal or organic base to form salts. Alkali and alkaline earth metals, heavy metals, amines and quaternary ammonium compounds may be used. Preferred are: Na, Li, K, Ca, Ba, Sr, Mg, Zn, Al, Cr, Co, Ni primary and secondary amines and the like.

To illustrate the pronounced improvement obtained in lubricating compositions by the addition of reaction products of this invention the following test data is given:

Compositions of this invention were evaluated as extreme pressure agents by use of the four-ball extreme pressure lubricating tester similar in principle to the Boerlage apparatus described in the magazine, Engineering, volume 136, July 14, 1933. This apparatus comprises four steel balls arranged in pyramid formation. The top ball is rotated by spindles against the three bottom balls which are clamped in a stationary ball holder. The balls are immersed in the composition to be tested. Tests were run under conditions indicated in the table and compared with other outstanding extreme pressure agents.

FOUR-BALL, E. P. LUBRICANT TESTER ON ADDITIVES  
IN SAE 90 OIL

[Fixed conditions: One-minute tests at 1500 R. p. m.]

| 5  | Additive                                                                                                                              | Am't,<br>Per<br>Cent<br>wt. | Seizure<br>Load,<br>in Kg. | Welding<br>Load,<br>in Kg. | Sear Di-<br>ameter,<br>in mm.<br>at 300<br>Kg. load |
|----|---------------------------------------------------------------------------------------------------------------------------------------|-----------------------------|----------------------------|----------------------------|-----------------------------------------------------|
| 10 | 1 None .....                                                                                                                          |                             | 50                         | 140                        | 4.2 at 120<br>Kg.                                   |
|    | 2 Benzoyl peroxide<br>catalyzed reaction<br>product of isophorone<br>bottoms and $CCl_4$ .                                            | 10                          | 80                         | 400                        | 2.6.                                                |
| 15 | 3 Benzoyl peroxide<br>catalyzed cracked<br>wax olefins and<br>$CCl_4$ .                                                               | 10                          | 60-80                      | 400                        | 3.1.                                                |
|    | 4 Di-tertiary butyl<br>peroxide catalyzed<br>hexadecene-1 with<br>dichloroacetic<br>acid.                                             | 10                          | 60-80                      | >700                       | 1.0.                                                |
| 20 | 5 Benzoyl peroxide<br>catalyzed reaction<br>product of isophorone<br>bottoms and<br>$CCl_4$ after treat-<br>ment with $H_2S-NH_4HS$ . | 10                          | 80-100                     | 700                        | 1.9.                                                |
|    | 6 Benzoyl peroxide<br>catalyzed cracked<br>wax olefins and<br>$CCl_4$ after treat-<br>ment with $H_2S-NH_4HS$ .                       | 10                          | 80-100                     | 700                        | 1.5.                                                |
| 30 | 7 Diterbutyl perox-<br>ide catalyzed, ce-<br>tene and dichloro-<br>acetic acid after<br>treatment with<br>$H_2S-NH_4HS$ .             | 10                          | 80-100                     | >700                       | 1.0.                                                |

In addition to the above properties the addition of reaction products of this invention to mineral lubricating oils inhibits lacquer formation in engines operating under the most adverse conditions. Also reaction product of this invention can be used as valuable constituents of heavy duty oils, motor oils, diesel oils, aviation oils, turbine oil, synthetic oils and the like because of their anti-corrosion, anti-oxidation, and anti-wear properties. Besides their utility as lubricating oil additives, reaction products of this invention are useful as anti-oxidants for natural and synthetic rubber and other organic materials which are subject to oxidation deterioration. The amount of additive used can be varied over wide limits but generally it is not necessary to use more than 5% by weight of the reaction product although amounts of as high as 10% can be used but preferably only between about 0.1 to 2.0% by weight is added to base lubricants.

Because of its synergistic effect the reaction product of this invention can be combined with other additives in lubricants, such as, blooming agents, pour point depressants or viscosity improvers, extreme pressure agents, anti-foaming agents and the like. Among the specific additives which can be used are oil-soluble detergents which include oil-soluble salts of various bases with detergent forming acids. Such bases include metal as well as organic bases. Metallic bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of, say, 10 to 30 carbon atoms, wool fat acids, paraffin wax acids (produced by oxidation of paraffin wax) chlorinated fatty acids, rosen acids, aromatic carboxylic acids including fatty acids, aromatic hydroxy fatty acids, paraf-

## 21

fin wax benzoic acids, various alkyl salicylic acids, phthalic acid monoesters, aromatic keto acids, aromatic ether acids, diphenols as di-(alkyl-phenol) sulfides and disulfides, methylene bis alkylphenols; sulfonic acids such as may be produced by treatment of alkyl aryl hydrocarbons or high boiling petroleum oils with sulfuric acid; sulfuric acid monoesters; phosphoric, arsonic and antimony acid mono and diesters, including the corresponding thiophosphoric, arsonic and antimony acids; phosphonic and arsonic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides such as lecithin and cephalin, certain fatty oils as rapeseed oils, volto-lized fatty or mineral oils and the like.

An excellent metallic detergent for the present purpose is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Anti-oxidants comprise several types, for example, alkyl phenols such as 2,4,6 trimethyl phenol, penta methyl-phenol, 2,4, dimethyl-6-tertiary-butyl phenol, 2,4-dimethyl-6-octyl phenol, 2,6-di-tertiary-butyl-4-methyl phenol, 2,4,6 tri-tertiary-butyl phenol and the like; amino phenols as benzyl amino phenols; amines such as dibutyl-phenylene diamine, diphenyl amine, phenyl - beta - naphthylamine, phenyl - alpha-naphthylamine, dinaphthyl amine.

Corrosion inhibitors or anti-rusting compounds may also be present, such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g. alpha cyano stearic acid).

Extreme pressure agents which may be used comprise: esters or phosphorus acids such as tri-aryl, alkyl hydroxy aryl, or aralkyl phosphates, thiophosphates or phosphites and the like; neutral aromatic sulfur compounds or relatively high boiling temperatures such as diaryl sulfides, diaryl disulfides, alkyl aryl disulfides, e. g. diphenyl sulfide, diphenol sulfide, dicrosol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g. sperm oil, jojoba oil, etc. in which the sulfur is strongly bonded; sulfurized long chain olefins such as may be obtained by dehydrogenation or cracking of wax; sulfurized phosphorized fatty oils or acids, phosphorus acid esters having sulfurized organic radicals, such as esters of phosphoric or phosphorus acids with sulfurized hydroxy fatty acids; chlorinated hydrocarbons, such as chlorinated paraffin, aromatic hydrocarbons, terpenes, mineral lubricating oil, etc.; or chlorinated esters of fatty acids containing the chlorine in position other than alpha position.

Additional ingredients may comprise oil-soluble urea or thiourea derivatives, e. g. urethanes, aliphonates, carbazides, carbazones, etc.; polyisobutylene polymers, unsaturated polymerized esters of fatty acids and monohydric alcohols and other high molecular weight oil-soluble com-

## 22

pounds. Depending upon the additive used and conditions under which it is used, the amount of additive used may vary from 0.01 to 2% or higher. However, substantial improvement is obtained by using amounts ranging from 0.1 to 0.5% in combination with phosphorous sulfide-unsaturated cyclic ketone reaction products of this invention.

It is to be understood that while the features of the invention have been described and illustrated in connection with certain specific examples, the invention, however, is not to be limited thereto or otherwise restricted, except by the prior art and the scope of the appended claims.

I claim as my invention:

1. A lubricant comprising a major amount of a mineral oil and a minor amount, sufficient to impart extreme pressure properties to said mineral oil, of a reaction product obtained by reacting an unsaturated organic compound selected from the group consisting of unsaturated cyclic ketone fractions containing at least 12 carbon atoms and monoolefinic aliphatic hydrocarbons containing at least 8 carbon atoms, with a poly-chlorinated saturated organic compound selected from the group consisting of polychlorinated hydrocarbons of from 1 to 2 carbon atoms and poly-chlorinated fatty acids of not more than 6 carbon atoms having at least 2 chlorine atoms which are separated from the carboxyl group of said acids by not more than 2 carbon atoms, in the mole ratio of from 1:1 to 1:4 respectively, in the presence of a peroxide catalyst under reflux conditions, and further treating said reaction product with hydrogen sulfide-ammonium hydrosulfide at above room temperature until saturated.

2. A lubricant comprising a major amount of a mineral oil and a minor amount of between about 0.1% and about 10.0% of a reaction product obtained by reacting an unsaturated cyclic ketone fraction containing at least 12 carbon atoms with carbon tetrachloride in the mole ratio of 1:1 to 1:4, respectively, in the presence of benzoyl peroxide under reflux conditions and further treating said reaction product with hydrogen sulfide—ammonium hydrosulfide at above room temperature until saturated.

3. A lubricant comprising a major amount of a mineral lubricating oil and a minor amount of between about 0.1% and about 10.0% of a reaction product obtained by reacting an isophorone bottoms fraction with carbon tetrachloride in the mole ratio of 1:1 to 1:4, respectively, in the presence of benzoyl peroxide under reflux conditions and further treating said reaction product with hydrogen sulfide-ammonium hydrosulfide at above room temperature until saturated.

4. A lubricant comprising a major amount of a mineral oil and a minor amount, sufficient to impart extreme pressure properties to said mineral oil, of a reaction product obtained by reacting an unsaturated organic compound selected from the group consisting of unsaturated cyclic ketone fractions containing at least 12 carbon atoms and monoolefinic aliphatic hydrocarbons containing at least 8 carbon atoms, with a poly-chlorinated saturated organic compound selected from the group consisting of polychlorinated hydrocarbons of from 1 to 2 carbon atoms and poly-chlorinated fatty acids of not more than 6 carbon atoms having at least 2 chlorine atoms which are separated from the carboxyl group of said acids by not more than 2 carbon atoms, in the mole ratio of from 1:1 to 1:4 respectively, in the presence of a peroxide catalyst under reflux conditions.

## 23

5. The composition of claim 4 wherein the unsaturated organic compound is an isophorone bottoms fraction.

6. The composition of claim 4 wherein the unsaturated organic compound is a cracked wax olefin.

7. The composition of claim 4 wherein the unsaturated organic compound is hexadecene-1.

8. The composition of claim 4 wherein the poly-chlorinated saturated organic compound is carbon tetrachloride.

9. The composition of claim 4 wherein the poly-chlorinated saturated organic compound is dichloroacetic acid.

10. A lubricant comprising a major amount of a mineral oil and a minor amount of between about 0.1% and about 10.0% of a reaction product obtained by reacting an unsaturated cyclic ketone fraction containing at least 12 carbon atoms with carbon tetrachloride in the mole ratio of 1:1 to 1:4, respectively, in the presence of benzoyl peroxide under reflux conditions.

11. A lubricant comprising a major amount of a mineral lubricating oil and a minor amount of

15

20

## 24

between about 0.1% and about 10.0% of a reaction product obtained by reacting an isophorone bottoms fraction with carbon tetrachloride in the mole ratio of 1:1 to 1:4, respectively, in the presence of benzoyl peroxide under reflux conditions.

12. A lubricant comprising a major amount of a mineral lubricating oil and a minor amount of between about 0.1% and about 10% of a reaction product obtained by reacting hexadecene-1 with dichloroacetic acid in the mole ratio of 0.5 to 2 respectively, in the presence of tertiary butyl peroxide under reflux conditions.

DAVID E. ADELSON.

## REFERENCES CITED

The following references are of record in the file of this patent:

## UNITED STATES PATENTS

| Number    | Name               | Date          |
|-----------|--------------------|---------------|
| 2,121,825 | Prutton            | June 28, 1938 |
| 2,197,781 | Badertscher et al. | Apr. 23, 1940 |
| 2,259,934 | Huijser et al.     | Oct. 21, 1941 |